

# UNITED STATES PATENT OFFICE.

WALTER O. SNELLING, OF ALLENTOWN, PENNSYLVANIA, ASSIGNOR, BY MESNE ASSIGNMENTS, TO TROJAN POWDER COMPANY, OF NEW YORK, N. Y., A CORPORATION OF NEW YORK.

## NITROSTARCH EXPLOSIVE.

1,386,437.

Specification of Letters Patent.

Patented Aug. 2, 1921.

No Drawing.

Application filed October 3, 1918. Serial No. 256,736.

To all whom it may concern:

Be it known that I, WALTER O. SNELLING, a citizen of the United States, and resident of Allentown, Lehigh county, Pennsylvania, 5 have invented certain Improvements in Nitrostarch Explosives, of which the following is a specification.

My invention relates to nitro-starch explosives, and its object is the production of 10 an explosive which will have great strength and at the same time be relatively insensitive to blows or friction. This combination of qualities is essential or desirable in certain classes of military explosives, for example for use as an explosive charge in 15 drop-bombs, and sea-mines, and for other uses.

Nitro-starch is itself a powerful explosive, and its strength is not materially decreased by the presence of a limited amount 20 of water. The water does not prevent detonation by an initial detonating means of sufficient strength, and owing to the intense heat produced at the instant of explosion, 25 the water present serves to increase the volume of gas which is produced. The presence of water in sufficient quantity to thoroughly wet the nitro-starch grains has the effect of rendering the explosive relatively 30 insensitive to blows or friction.

As however the water will evaporate when the wet nitro-starch is exposed to the air, the properties of the explosive mixture will rapidly change under the conditions incident to practical use. To avoid this, I mix 35 with the nitro-starch and water, in suitable proportions, a substance soluble in water and having sufficient affinity therefor to prevent ready evaporation of the water when 40 the mixture is exposed to the air, and I have discovered that in this manner highly useful explosives can be prepared having both the required strength and insensitiveness to 45 blows or friction.

I have found both inorganic and organic substances possessing the required hygroscopicity for the purpose stated. Examples 50 of inorganic salts are calcium chlorid and magnesium chlorid. As however these salts are explosively inert, and to obtain maximum strength it is desirable that no inert material should be present, I prefer to use a salt which is not only highly deliquescent, but which through its decomposition upon 55 detonation of the mixture, adds to the

strength of the explosive. As active inorganic agents, I instance the nitrates of ammonium, calcium, iron and lithium, which are highly hygroscopic and particularly well adapted to the purpose of my invention. Ammonium nitrate is the salt preferred.

Of organic materials suitable to the practice of my invention, dextrose and levulose have been found to be quite satisfactory, 65 either alone or admixed. Ordinary "invert sugar" serves very well, and commercial glucose is satisfactory. Other organic materials possessing sufficient hydroscopicity may be employed.

By varying the proportions of the several ingredients referred to, the physical characteristics of the explosive can be regulated as desired, to suit different purposes. For example, with a mixture containing 50% 75 nitro-starch, the deliquescent ingredient, say ammonium nitrate may represent 40% and the water 10%. This mixture is soft and plastic. A mixture containing 50% 80 nitro-starch, 45% ammonium nitrate and 5% of water, is quite dry, while one containing 50% nitro-starch, 37% ammonium nitrate, and 13% of water, is of semi-fluid consistency.

With mixtures containing a higher percentage of nitro-starch, as from 60% to 75%, the ammonium nitrate and water will represent from 40% to 25%, and of the solution of ammonium nitrate in water, less than 65% should be ammonium nitrate. In 90 such mixture the percentage of water is preferably more than 10% of the entire mixture, and in some cases can be more than 15%. For example, useful mixtures may be made in which the nitro-starch represents 95 60%, the ammonium nitrate somewhat less than 25%, and the water somewhat more than 15%; and nitro-starch 75%, ammonium nitrate somewhat less than 15% and water somewhat more than 10%. In 100 any event, to accomplish the desired purpose, the water should be in excess of 5% of the entire mixture. As at ordinary room temperature the water will not hold in solution more than approximately double its 105 weight of ammonium nitrate, it will be apparent that in some of the examples given the water will not be sufficient to hold in solution the entire amount of deliquescent salt present, but as in any event the water 110

present will be in excess of 5% of the total mixture, it will be sufficient to hold in solution a substantial amount of the deliquescent salt.

5 The proportions given for ammonium nitrate apply substantially with other hygroscopic ingredients employed for the same purpose, including those herein specifically named.

10 In the preparation of nitro-starch explosives according to my invention, I may directly mix together the three constituents in suitable proportions, using any type of mixer which will insure thorough incorporation, or

15 I may add together the water and the water soluble ingredient to obtain a concentrated solution, and this solution may then be added to the nitro-starch with proper incorporation.

20 It will be understood that instead of a single deliquescent material, I can use a combination of such materials. For example, the deliquescence of ammonium nitrate can be increased by the addition thereto of a small amount—say 1%—of a related deliquescent salt, such as lithium nitrate or sodium nitrate.

25 It will also be understood that in utilizing the explosive described, it can be incorporated with a suitable carbonaceous or combustible ingredient, in accordance with the practice in this art.

30 A characteristic of explosives made in accordance with my invention is their great strength, particularly their exceptional shattering strength and their relatively great insensitiveness. Their insensitiveness is due to the fact that the nitro-starch grains are thoroughly wet with the solution of the deliquescent material in water, and the action of the deliquescent material prevents the ready evaporation of the water from any exposed surface of the material. The exceptional strength which these explosives show is due

35 to the fact that nitro-starch is capable of detonating, even in the wet condition, that this nitro-starch is capable of bringing about the simultaneous detonation of the wet ammonium nitrate in those explosives in which

40 ammonium nitrate is the deliquescent agent used, and that even the water which is present in the mixture causes an increased gas volume at the moment of detonation owing to the intense heat produced at the time of

45 explosion, all of the constituents thus assisting in the production of a very great gas volume at the moment of explosion.

50 Although I have described certain specific mixtures of nitro-starch, water and water soluble materials having affinity for water, I do not wish in the broader aspect of the invention, to be limited to the hygroscopic materials specified, nor proportions named, since my invention is broadly applicable to explosives containing nitro-starch, a deliquescent

material, and water, where water is present in such amount as to be capable of holding in solution a substantial amount of the water soluble material.

55 I claim:

1. An explosive comprising nitro-starch, a deliquescent salt, and sufficient water to hold in solution a substantial amount of the deliquescent salt.

2. A nitro-starch explosive comprising nitro-starch maintained in wet condition by the addition of water containing a dissolved salt having great affinity for water.

3. A nitro-starch explosive containing water, and an ingredient having sufficient affinity for water to prevent its ready evaporation through exposure to air.

4. A nitro-starch explosive containing a saturated solution of a deliquescent salt.

5. A nitro-starch explosive comprising 50% of nitro-starch, 40% of ammonium nitrate and 10% of water.

6. A nitro-starch explosive comprising nitro-starch, a deliquescent nitrate, sufficient water to hold a substantial amount of the deliquescent nitrate in solution, and a suitable carbonaceous or combustible ingredient.

7. A nitro-starch explosive comprising nitro-starch, a saturated solution of an inorganic nitrate, and combustible constituent.

8. An explosive consisting of nitro-starch containing water sufficient to render it safe in handling, but insufficient to prevent its detonation, substantially as described.

9. An explosive consisting of nitro-starch containing a substantial percentage of water and ammonium nitrate, substantially as described.

10. An explosive consisting of nitro-starch than 10% of ammonium nitrate, substantially as described.

11. An explosive consisting of nitro-starch containing more than 10% of water and more than 10% of ammonium nitrate, substantially as described.

12. An explosive consisting of approximately 50% of nitro-starch, more than 10% of ammonium nitrate, and approximately 15% of water.

13. An explosive consisting of 60% to 75% of nitro-starch and from 25% to 40% of a solution of ammonium nitrate in water, substantially as described.

14. An explosive consisting of 60% to 75% of nitro-starch and from 25% to 40% of a solution of ammonium nitrate in water, said solution containing less than 65% of ammonium nitrate, substantially as described.

15. An explosive comprising nitro-starch and a sufficient amount of an unsaturated solution of ammonium nitrate in water to render the explosive non-inflammable.

WALTER O. SNELLING

Correction in Letters Patent No. 1,386,437.

It is hereby certified that in Letters Patent No. 1,386,437, granted August 2, 1921, upon the application of Walter O. Snelling, of Allentown, Pennsylvania, for an improvement in "Nitrostarch Explosives," an error appears in the printed specification requiring correction as follows: Page 2, strike out lines 104 to 106, comprising present claim 10 and insert the following as claim 10:

*10. An explosive consisting of nitrostarch containing more than 10% of water, substantially as described.;*

and that the said Letters Patent should be read with this correction therein that the same may conform to the record of the case in the Patent Office.

Signed and sealed this 11th day of October A. D., 1921.

[SEAL.]

WM. A. KINNAN,  
*Acting Commissioner of Patents.*